

## UNITED STATES PATENT OFFICE

2,002,932

STEEL FOR RAILROAD RAILS, WHEEL  
TIRES, PLANK PILES, AND OTHER  
OBJECTSHerbert Buchholz, Dortmund, Germany, assignor  
to the firm Vereinigte Stahlwerke Aktiengesell-  
schaft, Dusseldorf, GermanyNo Drawing. Application December 11, 1931,  
Serial No. 580,500. In Germany December 12,  
1930

2 Claims. (CL. 75—1)

This invention relates to a steel suitable for objects subjected to heavy wear.

The following fundamental requirements have to be met in the case of railroad rails:

- 5 1. The rails must have such a great mechanical strength that they are able to furnish sufficient resistance to stresses during service caused by wheel pressure, shocks and the like. For this purpose an adequately high elastic limit is necessary, in order to avoid the rails spreading under the wheel pressure, moreover an adequately high resistance to repeated shock stresses is also required, that is to say, a high resistance to impact stresses and prolonged stresses. Experience has shown that these requirements were first met by 10 steels having a high elastic limit and good toughness together with a moderate tensile strength.
2. The resistance to wear of the rails must be so great, that the least possible loss due to wear 15 takes place under the action of the rolling and sliding friction of the wheels travelling thereover.
- In addition to the technical requirements the question of economy is also of importance. The manufacture of the rails on the mass production 20 scale naturally entails the use of processes permitting the manufacture of a cheap steel. This condition is fulfilled in the first place by the Thomas-Gilchrist process and secondly by a suitable modification of the open-hearth process.
- 25 30. Information as to the properties which are of importance in the practical behaviour of the steel is furnished by the examination under the specification for the contract. This examination also extends to ascertaining whether the steel possesses adequate resistance to impact by means of the rail-impact test and proving whether the steel is sufficiently hard and strong mechanically by measuring the Brinell hardness or by means of the draw-test.
- 40 40. It is difficult to fulfil these manifold requirements without detrimentally affecting the other properties to a certain extent. The requirements as regards high toughness together with high mechanical strength counteract one another to a certain extent. The requirement as regards high 45 resistance to wear cannot be attained in view of the foregoing two criteria, since resistance to wear does not run parallel in any way to hardness, elastic limit or tensile strength.
- 50 50. It is therefore a question in view of the practical requirements of the case under consideration to evolve an optimum hardness, elastic limit, toughness and resistance to wear with the maximum economy. The means of effecting this are 55 various. It is well known that the tensile strength

and elastic limit may be increased by increasing the carbon content, the manganese content, the silicon content and also by the addition of other elements such as chromium, nickel and the like, the latter however not coming into consideration in the present case for economic reasons.

5 It is also known that increasing the content of manganese and also that of phosphorus increases the resistance to wear. Nevertheless a considerable increase in practice of the resistance to wear can only be produced by adding manganese in such quantities that the toughness (determined by the elongation during the fracture test, behaviour during the impact test and the notch-bar toughness) begins to decrease too rapidly. Hitherto no use at all could be made of the effect of the phosphorus increasing the resistance to wear, since, in the usual composition of the rails having phosphorus contents below about 0.08% practically no noticeable influence occurs and any increase of the phosphorus content above 0.1% 10 renders the rails too brittle, that is to say, too sensitive to shocks. For these reasons hitherto the steel works kept the phosphorus content at about 0.08% as the upper limit.

15 25 Tests made by the applicant have now shown that the property of phosphorus of increasing the resistance to wear of these steels can be made possible by adding this element in quantities of 0.08% and more and at the same time considerably reducing the carbon content so that it amounts to between 0.05 and 0.20% and maintaining the other constituents of the steel, particularly the manganese, within proper limits as hereafter specified. This steel intended for 30 rails complies to the fullest extent with all the requirements herein set forth at the outset. The very stringent impact test of the German State Railway Company which is accepted as the authority for practical service is passed in a fully 35 satisfactory manner, and on making the test more severe the rails only fracture after 6 or more blows usually after sagging to the extent of more than 140 mms. The elastic limit is sufficiently high, being more than 36 kg. per mm., to avoid 40 the rails spreading even when the wheel pressure is increased and the elongation and the notch-bar-toughness are of such a high order that there is no danger of the rail being affected detrimentally by impact or shocks. The resistance to wear 45 is increased to such a great extent by the combined action of manganese and phosphorus, that this steel can be compared directly with the steel rails which are known to be resistant to wear and which possess a tensile strength of more than 50

55

75 kg. per mm., the elongation however and in particular the notch-bar toughness of the steel of the present invention being greater than in the ordinary steel for rails having this strength. In order to bring about this object it is necessary to keep the carbon content low and if possible below 0.20%, the manganese content being kept within the limit of about 0.6 to 1.6% and the phosphorus being above 0.08% up to about 0.25% whilst the silicon content amounts to between 0.1% and 0.6% and the copper content to about 0.25 to 1.0%.

By said small content of copper the uniformity of the structure and the mechanical strength properties of this steel is increased. The copper content as is known also increases the resistance to corrosion and rusting of the steel, which is of considerable importance in service when the steel is used in the presence of corrosive media for example when the rails are laid in tunnels.

20 The steel may contain in addition thereto the usual accompanying elements, but if sulphur is present the content thereof shall be preferably kept low so as to lie from trace to about 0.12%.

The balance of the alloy consists substantially 25 of iron. It may be possible, however, to use some further alloying additions in known quantities and for known purposes. Such further alloying elements are comprised by the term "the balance substantially iron", provided, however, that the character of the alloy as described is not materially altered by such further additions and that the elements mentioned are present in the amounts specified.

30 The tensile strength properties and the resistance to wear of such rails were determined exhaustively from a large number of melts, the apparatus of Spindel and Mohr and Federhaff being employed for determining the resistance to wear.

Examples of the results of several tests on rail 40 melts are given in the following table.

The impact test prescribed by the German State Railway in their specification for steel was passed by these rails altogether in a very satisfactory manner, and even when this test was made more stringent, fracture only occurred after ordinary carbon steel rails having a tensile strength of 70 or 80 kg. per sq. mm. had already broken under the test. As may moreover be seen from the table resistance to wear is also considerably higher than that of other rails of the 10 same mechanical strength, values being shown which are only obtainable in carbon steel rails having a tensile strength of about 85 kg. per sq. mm.

When considering the results of the wear test 15 on the Mohr and Federhaff machines it should be mentioned that from practical experience rails having a decrease in weight during the test of less than 1.1 grams are termed "wear resistant". The rails produced according to the process of 20 the present invention exhibit throughout a decrease in weight of below 1.1 gram.

The permanent resistance to bending which is also important for practical service was ascertained by means of a plurality of tests on the 25 Schenck permanent bending machine, under loads of at least 30 kg. per sq. mm. and on the average of 34 kg. per sq. mm. Even when testing test pieces which were submitted to twists, values higher than 27 kg. per sq. mm. were invariably obtained. The steel thus possesses very high permanent strength at the same time very low notch-bar sensitivity during oscillatory 30 stresses.

Already in the year 1884 a report was made 35 (Tetmajer, Stahl und Eisen 4 (1884) pp. 608 to 613) on similar tests conducted with a view to producing a steel for rails from the Bessemer converter. The carbon content of these rails was reduced to about 0.2%, and the phosphorus 40

TABLE  
Composition and strength properties of rails S49

| 45     | Steel                      | Chemical composition |      |      |      |      |       | Strength properties |                  |                |                            |                                   | Wear                                  |                                          |     |
|--------|----------------------------|----------------------|------|------|------|------|-------|---------------------|------------------|----------------|----------------------------|-----------------------------------|---------------------------------------|------------------------------------------|-----|
|        |                            | C                    | Si   | Mn   | P    | Cu   | Cr    | Elastic limit       | Tensile strength | Elongation S10 | Reduction of cross section | Notched bar tenacity <sup>1</sup> | Spindel length of cut in <sup>2</sup> | Mohr and Federhaff decrease <sup>3</sup> |     |
| 45     |                            |                      |      |      |      |      |       |                     |                  |                |                            |                                   |                                       |                                          |     |
| 50     |                            |                      |      |      |      |      |       |                     |                  |                |                            |                                   |                                       |                                          |     |
| 1..... | Carbon steel. (Comparison) | 0.36                 | 0.02 | 0.74 | 0.08 | 0.02 | 0.02  | 37                  | 67               | 18             | 18                         | 3                                 | 43                                    | 1.4                                      |     |
| 55     | 2.....                     | 0.42                 | 0.15 | 0.93 | 0.05 | 0.06 | ----- | 40                  | 78               | 15             | 16                         | 2                                 | 41                                    | 1.1                                      |     |
| 55     | 3.....                     | P-Mn steel.          | 0.11 | 0.60 | 1.50 | 0.11 | 0.50  | -----               | 43               | 61             | 24                         | 58                                | 6                                     | 30                                       | 0.9 |
| 60     | 4.....                     |                      | 0.07 | 0.25 | 1.52 | 0.09 | 0.45  | 0.6                 | 42               | 58             | 22                         | 52                                | 11                                    | 28                                       | 0.8 |
| 60     | 5.....                     |                      | 0.14 | 0.40 | 1.20 | 0.16 | 0.40  | -----               | 43               | 62             | 19                         | 54                                | 5                                     | 38                                       | 0.8 |
| 60     | 6.....                     |                      | 0.10 | 0.40 | 1.30 | 0.18 | 0.40  | -----               | 45               | 62             | 17                         | 48                                | 6                                     | 27                                       | 0.7 |
| 60     | 7.....                     |                      | 0.12 | 0.45 | 1.30 | 0.12 | 0.50  | 0.15                | 42               | 50             | 23                         | 50                                | 5                                     | 40                                       | 0.9 |

<sup>1</sup> Form of test piece 10x10x60 with a circular notch 5 mm. deep 2 mm.  $\phi$ .

<sup>2</sup> Length of cut as the average of 4 grinding cuts under a pressure of 5 kg., 250 complete revolutions n=25.

<sup>3</sup> Decrease after 200,000 revolutions under an applied pressure of 100 kg., 1% slip, 425 revolutions per minute.

65 In spite of the relatively low carbon content the elastic limit of the steel is above 40 kg. per sq. mm., i. e. it possesses values which could only be produced in an ordinary steel having a carbon content of more than 0.5%.

70 The tensile strength amounts at the same time to about 60 kg. per sq. mm. the elongation to more than 16% and on the average 20%, being thus very considerably higher than that of a carbon steel of the same or even higher tensile strength.

content was increased to over 0.1%, the silicon content being increased at the same time. The tests were however fruitless, since it is expressly emphasized that these rails were brittle and showed a tendency to form cracks.

75 Similar considerations as has been mentioned in the foregoing for rails also apply when carrying out the process for the production of wheel tires plank-piles and particularly for sea walls and other steel parts which are subjected to wear.

Having now particularly described and ascer-

tained the nature of my said invention and in what manner the same is to be performed, I declare that what I claim is:

1. A steel for railroad rails, wheel tires, plank-piles and other objects which are subjected to heavy wear, said steel containing about 0.05 to 0.20% of carbon, about 0.08 to 0.25% of phosphorus, about 0.1 to 0.6% of silicon, about 0.6 to 1.6% of manganese and about 0.25 to 1% of copper, the balance substantially iron.

10 per and the balance substantially iron.

2. A steel for railroad rails, wheel tires, plank-piles and other objects, which are subjected to heavy wear, with a sulphur content of from trace to about 0.12%, said steel containing about 0.05 to 0.20% of carbon, about 0.08 to 0.25% phosphorus, about 0.1 to 0.6% of silicon, about 0.6 to 1.6% of manganese and about 0.25 to 1% of copper, the balance consisting substantially of iron.

HERBERT BUCHHOLTZ. 10